

## UNITED STATES PATENT OFFICE.

LUTHER FERSTER AND CLARENCE FERSTER, OF ROCK ISLAND, ILLINOIS.

## RAZOR STROP AND THE PREPARATION THEREOF.

No Drawing.

Application filed October 4, 1924. Serial No. 741,760.

Our invention has reference to razor strops, and the method of preparing the same for use, the purpose thereof being to produce a strop which will possess a maximum of efficiency, which will be durable, and which will not be affected by atmospheric conditions, such as will ordinarily cause the strop to buckle, and get out of shape for use.

10 The invention is more specially designed for use in a strop formed of canvas or other fibrous material, and the preparation thereof consists in applying thereto an emulsion of a novel character, and adapted to act

15 as a filler. The strop is thereby prepared to receive another and different emulsion, also of a novel character, and which forms a coat or dressing therefor. The two emulsions, or compounds, are dependent to a

20 large extent upon each other, but another preparation might be substituted for the filler emulsion, and the dressing compound act as efficiently therewith.

The first mentioned, or filler emulsion, is made up of the following ingredients, in approximately the proportions mentioned, to wit: water, 16 ounces; wood oil, 8 ounces; cotton-seed oil, 8 ounces; commercial soap, 7 drams and 20 grains. The strop to be prepared is saturated with the compound formed by thoroughly mixing said ingredients, the emulsion penetrating all of the fibers contained in the strop, and acting as a perfect filler therefor, fully excluding any other compound, and preparing the strop to receive the dressing coat, which is made up of the following ingredients, also thoroughly mixed with each other, to wit:

Water, 16 ounces; wood-oil, 8 ounces;

olive oil 2 ounces; calcium carbonate, 1 40 and  $\frac{1}{4}$  ounces; zinc oxide, 1 and  $\frac{1}{4}$  ounces; white bees-wax, 3 drams and 20 grains; commercial soap, 7 drams and 20 grains. This second emulsion is applied to the strop in the usual manner for forming a dressing 45 thereon, to be used in putting an edge on the blade of a razor. The strop forms the base, and, when provided with the filler compound, serves as the ground for the final application, or dressing coat. In the 50 stropping operation the strop also serves as a supporting member, to receive the strokes of the razor, and is also a carrier for the compounds which have been applied thereto.

It will be evident that changes can be 55 made in the proportions of the various ingredients in either of the compounds, within reasonable limits, without departing from the scope or usefulness thereof. A strop formed in the above described manner will 60 always be soft and pliable, and specially fitted for the use for which it is intended.

What we claim, and desire to secure by Letters Patent, is:—

In a razor strop preparation, a dressing emulsion, consisting of the following ingredients thoroughly mixed together, and in approximately the proportions named, to wit: water, 16 ounces; wood oil, 8 ounces; olive oil, 2 ounces; calcium carbonate, 1 and  $\frac{1}{4}$  ounces; zinc oxide, 1 and  $\frac{1}{4}$  ounces; white bees-wax, 3 drams and 20 grains; and commercial soap, 7 drams and 20 grains.

In testimony whereof we affix our signatures.

LUTHER FERSTER.  
CLARENCE FERSTER.